

# United States Patent [19]

Caule et al.

[ 19 ]

[11] 3.811.874

[45] May 21, 1974

- [54] **OXIDATION RESISTANT IRON BASE ALLOY**

[75] Inventors: **Elmer J. Caule**, New Haven; **Philip R. Sperry**, North Haven; **Michael J. Pryor**, Woodbridge; **James A. Ford**, North Haven, all of Conn.

[73] Assignee: **Olin Corporation**, New Haven, Conn.

[22] Filed: **Aug. 13, 1971**

[21] Appl. No.: **171,432**

#### Related U.S. Application Data

- [63] Continuation-in-part of Ser. Nos. 66,866, Aug. 25, 1970, Pat. No. 3,730,779, and Ser. No. 750,991, Aug. 7, 1968, abandoned.

[52] U.S. Cl. .... 75/124

[51] Int. Cl. .... C22c 39/54

[58] Field of Search .... 75/124

## [56] References Cited

UNITED STATES PATENTS

- 851,635 4/1901 Hadfield ..... 75/124

- |           |         |                |        |
|-----------|---------|----------------|--------|
| 1,128,726 | 2/1965  | Rubel.....     | 75/124 |
| 2,835,570 | 5/1958  | Klaybor .....  | 75/124 |
| 3,207,637 | 9/1965  | Matuschka..... | 75/124 |
| 422,403   | 3/1880  | Hadfield ..... | 75/124 |
| 1,995,562 | 3/1935  | Browne.....    | 75/124 |
| 2,140,237 | 12/1938 | Leitneu.....   | 75/124 |
| 3,431,101 | 3/1969  | Kunitake.....  | 75/124 |

*Primary Examiner*—Hyland Bizot

*Attorney, Agent, or Firm—Robert H. Bachman*

[57]

## ABSTRACT

Iron base alloys are disclosed containing certain alloying additions, which alloys exhibit unique and unexpectedly low weight gains when exposed to oxidizing environments. One of the major advantages of the alloys of the present invention lies in their moderate cost, especially as compared to other oxidation resistant iron base alloys, such as the various grades of stainless steel. The oxidation resistance of the alloys of the present invention is imparted through the formation of a tenacious, compact oxide film.

## 2 Claims, 4 Drawing Figures



PATENTED MAY 21 1974

3,811,874

SHEET 1 OF 4



FIG. 1

ELMER J. CAULE  
PHILIP R. SPERRY  
MICHAEL J. PRYOR  
JAMES A. FORD  
INVENTORS

BY *R. Bachman*  
ATTORNEY

SHEET 2 OF 4



FIG- 2

ELMER J. CAULE  
PHILIP R. SPERRY  
MICHAEL J. PRYOR  
JAMES A. FORD  
INVENTORS

BY *R.H. Bachman*  
ATTORNEY

PATENTED MAY 21 1974

3,811,874

SHEET 3 OF 4



FIG-3

INVENTORS:  
ELMER J. CAULE  
PHILIP R. SPERRY  
MICHAEL J. PRYOR  
JAMES A. FORD  
BY  
*R. Bachman*  
ATTORNEY

PATENTED MAY 21 1974

3,811,874

SHEET 4 OF 4



FIG-4

ELMER J. CAULE  
PHILIP R. SPERRY  
MICHAEL J. PRYOR  
JAMES A. FORD  
INVENTORS

BY *R. Bachman*  
ATTORNEY

## OXIDATION RESISTANT IRON BASE ALLOY

## CROSS REFERENCE TO RELATED APPLICATIONS

This application is a continuation-in-part of copending application Ser. No. 66,866 now U.S. Pat. No. 3,730,779, May 1, 1973 by Caule et al. for Oxidation Resistant Iron Base Alloy, filed Aug. 25, 1970, and copending application Ser. No. 750,991 now abandoned by Caule et al. for Oxidation Resistant Iron Base Alloy, filed Aug. 7, 1968.

## BACKGROUND OF THE INVENTION

It has long been an objective of the art to provide low cost iron base alloys with oxidation resistance superior to that exhibited by the stainless steels. Presently, the only known method for imparting such oxidation resistance resides in the formation of an adherent chromium oxide surface layer.

However, the provision of an adherent chromium oxide surface layer requires large amounts of chromium in solid solution in the matrix. It has been shown that at least 11 percent by weight of chromium is necessary to provide the very excellent oxidation resistance characteristics of stainless steels.

It has further been sought to provide low cost iron alloys with excellent corrosion resistance in ambient environments as compared to mild steel and the specially designed low alloy steels, such as Corten. One of the disadvantages of the mild steels and specially designed low alloy steels is their extensive production of red rust rundown.

Accordingly, it is a principal object of the present invention to provide a low cost iron base alloy having oxidation resistance comparable to or superior to that exhibited by the stainless steels.

It is a further object of the present invention to provide such iron alloys which do not rely on large amounts of chromium in solid solution for their oxidation resistance.

It is an additional object of the present invention to provide alloys as aforesaid which in addition are characterized by improved resistance to corrosion in ambient environments without the disadvantage of extensive red rust rundown.

Further objects and advantages of the present invention will appear from the ensuing specification.

## SUMMARY OF THE INVENTION

In accordance with the present invention it has been found that the foregoing objects and advantages may be readily achieved.

The present invention resides in an oxidation and tarnish resistant iron base alloy consisting essentially of (A) an alloying addition in an amount from 1 to 7 percent by weight selected from the group consisting of beryllium, aluminum, indium and gallium and (B) an alloying addition in an amount from 1 to 4 percent by weight selected from the group consisting of silicon and germanium.

The alloy of the present invention contains less than 0.25 percent copper. It has been found to be necessary to restrict the copper content in order to obtain the excellent oxidation resistance of the present invention.

The alloy of the present invention may contain phosphorus 0.04 percent max., sulfur 0.04 percent max.,

manganese up to 1.5 percent, carbon up to 2 percent and others up to 0.20 percent, balance iron.

The alloy of the present invention is further characterized by having a tenacious, compact substantially colorless and adherent film, which film contains iron plus one of the group (A) elements.

The alloy of the present invention has significantly greater oxidation resistance than stainless steels in a 300° to 1,000°C range and exhibits a decrease in weight gain with increasing temperature.

The alloys of the present invention achieve numerous surprising and unexpected advantages. For example, as shown in the instant specification, it has been found that an iron-aluminum-silicon alloy of the present invention exhibits oxidation weight gain on the order of 50 times less than experienced by stainless steels or other iron base alloys. Further advantages and surprising characteristics of the alloys of the present invention will appear from the ensuing specification.

## BRIEF DESCRIPTION OF THE DRAWINGS

In the drawings which form a part of the present specification,

FIG. 1 is a graph showing the oxidation weight gain of three alloys at various temperatures. Alloy 1 is an iron-3 percent aluminum — 2 percent silicon alloy of the present invention. Alloy 2 is type 301 stainless steel (iron-17 percent chromium — 7 percent nickel alloy). Alloy 3 is a comparative iron-3 percent aluminum — 2 percent silicon alloy containing 1.1 percent copper.

FIG. 2 is a ternary plot of iron-aluminum-silicon alloys of the present invention showing weight gains in micrograms per square centimeter after heating for 2 hours at 800°C. FIG. 2 also shows for comparison the weight gains of binary iron-silicon alloys and binary iron-aluminum alloys.

FIG. 3 is a graph showing oxidation weight gains at various temperatures for an iron-gallium-silicon alloy of the present invention.

FIG. 4 is a graph comparing the behavior of an iron-3 percent aluminum — 2 percent silicon alloy of the present invention with type 301 stainless steel in a wet oxidizing, sulfur dioxide atmosphere.

The drawings will be discussed in more detail in the ensuing specification.

## DETAILED DESCRIPTION

As indicated hereinabove, the alloys of the present invention have greatly improved oxidation and tarnish resistance. In fact, the oxidation resistance of the alloys of the present invention is significantly greater than that which is achieved by stainless steels in the temperature range from 300° to 1,000°C.

The surprising oxidation resistance of the alloys of the present invention is achieved by the addition of specified alloying ingredients and by the formation of a tenacious, compact substantially colorless and adherent oxide film.

The alloy of the present invention contains an alloying addition in the amount from 1 to 7 percent selected from the group consisting of beryllium, aluminum, indium and gallium.

The alloy of the present invention also contains an alloying addition in the amount from 1 to 4 percent selected from the group consisting of silicon and germanium.

Representative specific combinations of materials are the following compositions: 3 percent beryllium — 2 percent silicon; 3 percent indium — 2 percent silicon; 3 percent gallium — 2 percent silicon; 3 percent aluminum — 2 percent germanium; and 3 percent aluminum — 2 percent silicon.

The alloys of the present invention unexpectedly show a reversal in the plot of weight gain against temperature as will be apparent from a consideration of the drawings which form a part of the present specification. This is believed to result from the formation of a tenacious, compact substantially colorless and adherent oxide film which contains iron plus one of the elements beryllium, aluminum, indium and gallium. For example, in the case where aluminum is used, there is formed aluminum oxide and a complex of the type  $FeO \cdot Al_2O_3$ . In the case where gallium is utilized, there is formed  $Ga_2O_4$  and a complex of the type  $FeO \cdot Ga_2O_3$ . The elements silicon and germanium are believed to stimulate the formation of oxides of this type.

In addition to the foregoing, it has been found that the copper content should be restricted to a maximum of 0.25 percent. It has been found to be necessary to restrict the copper content in order to obtain the excellent oxidation resistance of the present invention. In fact, it has been found that the higher copper contents yield poor oxidation resistance at both the lower and higher temperatures.

In addition to the foregoing, the alloys of the present invention may contain phosphorus 0.04 percent max., sulfur 0.04 percent max., manganese up to 1.5 percent and preferably up to 0.2 percent, others including nickel, molybdenum and vanadium and other alloying elements commonly present in low alloy steels may be present in an amount up to 0.20 percent. The carbon content may range as high as 2 percent for some applications requiring very high wear resistance. However, the carbon content is preferably not more than about 1 percent. Furthermore, the most preferred range of carbon is from 0.01 to 0.25 percent. It is expected that the latter range will have the most general application.

The iron base alloys of the present invention may be processed according to ordinary iron base alloy melting, casting, and hot and cold working procedures. It is an advantage of the present invention that the alloys of the present invention do not require specialized equipment or technology.

For example, the alloys of the present invention may be vacuum cast, homogenized, for example at 1,800°F, hot rolled to approximately 0.200", with a reheating to 1,800°F, if desired, scalped and cold rolled without interannealing to from 0.200" gage to 0.015" gage.

However, the alloy of the present invention does not require vacuum casting. Ordinary steel making procedures may be readily employed, as is well known in the art.

As indicated hereinabove, the alloys of the present invention are characterized by a great many highly desirable and in fact surprising characteristics. Particularly, the alloys of the present invention have surprising oxidation resistance, as has been discussed hereinabove. It is particularly significant that the alloys of the present invention achieve this surprising oxidation resistance while being considerably less expensive than alloys containing relatively large amounts of chromium, such as amounts of at least 5 percent and gener-

ally above 11 percent. For example, the commonly used stainless steel which contains approximately 18 percent chromium and 8 percent nickel.

Furthermore, if one first forms the film of the present invention, subsequently the materials exhibit no further weight gain. This is particularly significant. Thus, for example, it has been found that the alloys of the present invention are highly resistant to atmospheric oxidation and tarnishing after first being exposed to a high temperature air oxidation of from 5 minutes to 100 hours at 400° to 1,000°C and preferably 600° to 1,000°C. Thus, 2 hours at 800°C has been found to be very satisfactory.

The alloys of the present invention are characterized by the further advantage of excellent resistance to corrosion in ambient environments as compared to mild steel and specially designed low alloy steels, such as Corten. One of the disadvantages of the foregoing alloys is their extensive production of red rust rundown. On the other hand, the alloys of the present invention have shown as much as 50 to 75 percent less red rust rundown after one year of exposure.

It has also been found that the alloys of the present invention are highly resistant to contaminated atmospheres containing sulfur and/or water vapor and/or carbon monoxide-carbon dioxide combinations. These atmospheres are representative of most hydrocarbon combustion gases. The alloys of the present invention exhibit improved oxidation resistance in sulfur dioxide containing environments at elevated temperatures. In addition, if the alloys of the present invention are pre-treated in air at elevated temperatures, such as 800°C in order to first form the film of the present invention, the instant alloys show substantial improvement over, for example, type 301 stainless steel over the entire temperature range, when treated in wet oxidizing, sulfur dioxide environments. Surprisingly, the weight gain shown by the alloys of the present invention is essentially zero at from above about 450°C.

The present invention will be more readily understandable from a consideration of the following illustrative examples.

#### EXAMPLE I

Iron base alloys were prepared by the following method. The alloys were cast by the vacuum melting technique. The castings were soaked at 1,800°F for 2 hours and hot rolled to 0.60" in four passes. The materials were reheated and soaked at 1,800°F for an additional 1½ hours. Subsequently, the alloys were hot rolled to 0.20" in three passes. The hot rolled plates were scalped along both edges and top and bottom surfaces, leaving a finished gage of 0.17". The as-scalped plates were cold rolled to 0.015". All cold rolling was carried out without the benefit of further annealing.

#### EXAMPLE II

After the procedure of Example I, the surface of the materials were cleaned and chemically polished. The specimens were oxidized for 2 hours in a horizontal tube furnace open at both ends to the atmosphere. Specimens were placed in the hot furnace at the beginning of the run at various temperatures. The weight gains were determined by before and after weighing on a microbalance.

In this example, three alloy samples were studied having the composition indicated hereinbelow.

TABLE A

| Alloy | COMPOSITION |         |        |          |        |         | Iron |
|-------|-------------|---------|--------|----------|--------|---------|------|
|       | Aluminum    | Silicon | Copper | Chromium | Nickel |         |      |
| 1     | 3%          | 2%      | Nil    | —        | —      | Balance |      |
| 2*    | —           | —       | —      | 17%      | 7%     | Balance |      |
| 3     | 3%          | 2%      | 1.1%   | —        | —      | Balance |      |

\*Type 301 Stainless Steel

FIG. 1 shows the oxidation weight gain of Alloys 1, 2 and 3. It should be noted that Alloy 1, the alloy of the present invention exhibits a unique and unusual reversal in oxidation weight gain in the temperature range of 600° to 900°C. This is in distinct contrast to the oxidation weight gain exhibited by stainless steel type 301 (Alloy 2) over the same temperature range. Alloy 3 clearly shows that with higher copper contents there results poor oxidation resistance at both the lower and higher temperature ranges.

Alloy 1 as characterized by having a tenacious, compact substantially colorless and adherent oxide film. Upon examination, this film was found to contain  $\text{Al}_2\text{O}_3$  and a complex of the type of  $\text{FeO}\cdot\text{Al}_2\text{O}_3$ .

### EXAMPLE III

Example III compares the weight gains in micrograms per square centimeter of various iron-aluminum-silicon alloys of the present invention after the alloys were heated for 2 hours at 800°C. The materials were all prepared in a manner after Example I and treated in a manner after Example II.

The results are shown in FIG. 3 which is a ternary plot of the iron-aluminum-silicon alloys of the present invention. FIG. 2 also shows by comparison the weight gains of binary iron-silicon alloys and binary iron-aluminum alloys.

It is apparent from a consideration of FIG. 2 that the alloys of the present invention have much lower weight gains than the binary alloys. In fact, from this data, it is apparent that weight gains below 50 micrograms per square centimeter are assured for the 2 hour treatment at 800°C.

### EXAMPLE IV

In this example an alloy was prepared in a manner after Example I and processed in a manner after Example II, said alloy having the following composition: gallium-3 percent, silicon-2 percent, copper-nil, balance iron. The oxidation weight gains of this alloy over various temperatures are shown in FIG. 3. It should be noted that at the high temperatures this alloy exhibited

a weight gain substantially less than many types of stainless steels.

### EXAMPLE V

15 In this example the behavior of Alloy 1 above in a wet oxidizing  $\text{SO}_2$  atmosphere was compared with type 301 stainless steel in the same atmosphere. The results are shown in FIG. 4. It should be noted that above 700°C, the alloy of the present invention is clearly superior to 20 type 301 stainless steel.

### EXAMPLE VI

An alloy of the present invention was prepared in a manner after Example I and processed as in Example 25 II. The alloy had the following composition: aluminum-3 percent, germanium-2 percent, copper-nil, iron essentially balance. The alloy exhibited the tenacious film of the present invention and showed improved oxidation resistance at 750°C and above as compared to type 30 stainless steels.

This invention may be embodied in other forms or carried out in other ways without departing from the spirit or essential characteristics thereof. The present embodiment is therefore to be considered as in all respects illustrative and not restrictive, the scope of the invention being indicated by the appended claims, and all changes which come within the meaning and range of equivalency are intended to be embraced therein.

40 What is claimed is:

1. An oxidation and tarnish resistant iron base alloy consisting essentially of (A) an element in the amount from 1 to 7 percent selected from the group consisting of beryllium, aluminum, indium and gallium and (B) 45 germanium in an amount of from 1 to 4 percent, said alloy having a copper content of less than 0.25 percent, phosphorus, 0.04 percent max., sulfur 0.04 percent max., manganese up to 0.2 percent, carbon up to 1 percent, balance iron, said alloy having a tenacious, compact, substantially colorless and adherent oxide film containing a complex oxide which contains iron plus one of said group (A) elements, said alloy having improved oxidation resistance and exhibiting a decrease in weight gain with increasing temperature.

50 2. An iron base alloy according to claim 1 wherein said group (A) element is aluminum and said group (B) element is germanium.

\* \* \* \* \*